

Dec. 19, 1972

R. H. SPRAGUE

3,706,559

METHODS FOR MAKING POSITIVE FULL-COLOR DYE-TRANSFER PRINTS

Filed Feb. 27, 1969

ORIGINAL IMAGE: RED GREEN BLUE

COLOR NEGATIVE: CYAN MAGENTA YELLOW

EXPOSURE

RED SENSITIVE: — X X

GREEN SENSITIVE: X — X

BLUE SENSITIVE: X X —

DEVELOPMENT and TRANSFER

RED SENSITIVE: — CYAN CYAN

GREEN SENSITIVE: MAGENTA — MAGENTA

BLUE SENSITIVE: YELLOW YELLOW —

DYE TRANSFER PRINT: RED GREEN BLUE

FIG. 1.



FIG. 2.

ROBERT H. SPRAGUE  
INVENTOR.

BY

*W. Gary Goods*

ATTORNEY.

## 1

3,706,559

METHODS FOR MAKING POSITIVE FULL-COLOR  
DYE-TRANSFER PRINTSRobert H. Sprague, Chelmsford, Mass., assignor to  
Itek Corporation, Lexington, Mass.  
Filed Feb. 27, 1969, Ser. No. 802,954

Int. Cl. G03c 5/24

U.S. CL. 96—48 PD

9 Claims

## ABSTRACT OF THE DISCLOSURE

Methods are disclosed for making positive full-color dye-transfer prints by imagewise exposure, to a color negative, of photographic imaging media comprising a finely-divided photoconductor as the photosensitive agent. The exposed imaging media are developed, in the presence of a reducible metal ion, with couplers and developers forming cyan, magenta, or yellow dye images in radiation-exposed portions thereof. These dye images combine to reproduce the original image in a full-color print.

## BACKGROUND OF THE INVENTION

## (1) Field of the invention

This invention relates to methods for making positive full-color dye transfer prints and to multi-layer photographic imaging media for preparing such dye transfer prints.

## (2) Description of the prior art

U.S. Pat. No. 3,380,823 discloses photographic imaging media comprising a finely-divided photoconductor as the photosensitive agent. Exposure of such imaging media to actinic radiation such as visible or ultraviolet light activates the photoconductor, rendering it capable of effecting chemical reactions which can be utilized to develop a visible image. As taught in this patent and known in the art, the photoconductors of greatest utility for use in such imaging media are compounds formed between metals and elements of Group VI-A of the Periodic Table, e.g. oxides, sulfides, selenides and tellurides. Preferred materials from the point of view of color, light-sensitivity, ease of development, and the like are titanium dioxide and zinc oxide.

The latent image of activated photoconductor formed in such imaging media by imagewise exposure thereof can be suitably developed by applying image-forming materials to the media. Suitable image-forming materials include redox systems, for example systems containing reducible metal ions such as silver ions or other ions of noble metals at least as easily reducible as ionic copper. U.S. Pats. Nos. 3,227,551 and 3,243,294 teach color photographic diffusion-transfer processes employing ballasted couplers, present in silver halide imaging media, which form and/or release diffusible dyes during development.

## SUMMARY OF THE INVENTION

According to the present invention, a photographic imaging medium comprising a finely-divided photoconductor as the photosensitive agent, said photoconductor suitably being dispersed in a binder to form a photosensitive layer coated on a supporting substrate such as of paper, metal, glass, plastic, or the like, is exposed to

## 2

imaging radiation which activates the photoconductor in radiation-exposed areas. Those portions of the photographic medium containing activated photoconductor are next developed by contacting the exposed medium, in the presence of reducible metal ions, with a color-forming coupler and a photographic developer which in its oxidized form is reactive with said color coupler to form a dye. In those portions of the imaging medium in which the photoconductor has been activated by radiation, metal ions are reduced to form a deposit of free metal whereas the developer is oxidized and reacts with the coupler to form a dye.

For forming full color prints, three separate imaging media may be used respectively sensitized to red, green, and blue light and respectively forming cyan, magenta, and yellow dye images which are transferred in register to a receptor sheet to form a dye transfer print. In another embodiment of the invention, these photosensitive color-producing entities may form three layers of a single multi-layer medium.

Where separate media are employed to produce a full color print, the dye-forming developer and coupler may be present in the same development bath. They react to form dye when contacted with irradiated portions of the imaging medium in the presence of metal ion.

If the plural photosensitive entities necessary to produce a full color print comprise different layers of a single multi-layer imaging medium, appropriate ballasted couplers are suitably incorporated within the various layers. These couplers react with developer, at photo-activated sites and in the presence of a metal ion, to form and/or release diffusible dyes which are then transferred to a receptor sheet to form a positive dye transfer image.

To decrease fog which may appear in unexposed portions of a printing medium by reaction of metal ion with developer, a competing coupler may advantageously be incorporated into the radiation-sensitive layer or layers thereof. The competing coupler is capable of reacting with oxidized developer to form a non-diffusing compound. In unexposed areas, the competing coupler removes unwanted oxidized developer by formation of a non-diffusing compound, thus inhibiting fog formation. In exposed areas, where oxidized developer is plentifully present, the competing coupler does not consume enough of the developer to interfere with the production of a quality print by reaction of the oxidized developer with the regular coupler.

## DESCRIPTION OF PREFERRED EMBODIMENT

A better understanding of the present invention will be had by referring to the accompanying drawing, in which FIG. 1 is a schematic plan showing image and image-copy color relationships at various stages of a process for producing a dye transfer print according to the present invention; and FIG. 2 is an enlarged side view, in section, of a typical multi-layer photographic medium useful for the preparation of full-color dye transfer prints according to the present invention.

FIG. 1 shows that an original image comprising red, green and blue portions is reproduced in a color negative, e.g. a conventional silver halide color negative such as a "Kodacolor" negative, as a dye image respectively comprising cyan, magenta, and yellow portions.

As further suggested by the "Exposure" plan shown in FIG. 1, according to the present invention, a first, red-

sensitive, photographic imaging medium comprising a finely-divided photoconductor sensitized to red light is exposed to white light through such as color negative. The magenta and yellow portions of the negative transmit red light and expose the medium correspondingly (as indicated by "X" in the figure), but the medium remains unexposed wherever red-absorbing cyan dye is present in the color negative (i.e. wherever red was present in the original image).

A second medium comprising green-sensitized photoconductor is exposed to the color negative using white light. This activates the photoconductor in those portions of the medium corresponding to the green-transmitting cyan and yellow portions of the color negative.

Exposure of a third, blue-sensitive, imaging medium to white light through the color negative activates the photo-sensitive photoconductor of the medium only in those portions corresponding with cyan and magenta areas of the color negative, i.e. those areas of the negative which transmit blue light.

(The red, green, and blue-sensitive media mentioned above are suitably prepared by dispersing a finely-divided photoconductor such as finely-divided titanium dioxide in a binder such as gelatin, and coating a support layer such as paper or cellulose acetate with the mixture. The photoconductor is suitably sensitized to red, green, or blue light with cyanine and hemicyanine dyestuffs like those taught in Belgian Pat. 714,080.)

The exposed media, now containing radiation-activated photoconductor, are next developed in the presence of a reducible metal ion. Suitably, the exposed media are first contacted with an aqueous solution of an appropriate metal ion e.g. a solution of silver nitrate, and are then developed in a developing bath comprising a photographic developer and a coupler capable of reacting with oxidized developer to form a cyan, magenta, or yellow dye.

Thus, the exposed red-sensitive medium discussed above is suitably first contacted with a solution of aqueous silver nitrate and then developed in a bath comprising a photographic developer and a coupler reacting with oxidized developer to form a cyan dye. Where the photoconductor has been activated by exposure, metal ion is reduced and developer is oxidized and combines with the coupler to form cyan dye as shown in FIG. 1.

The exposed green-sensitive layer is developed with a second developing solution containing developer and a coupler forming a magenta dye, and the exposed blue-sensitive layer is separately developed with still another developer-coupler solution with formation of a yellow dye image in exposed areas.

As further suggested in FIG. 1, when the cyan, magenta, and yellow images respectively formed in the now-developed media are transferred in register to a receptor sheet, a positive print reproducing the pattern of reds, greens, and blues of the original image is obtained.

FIG. 2 of the accompanying drawing shows a photographic printing medium according to the present invention in which red-sensitive, green-sensitive, and blue-sensitive layers are present in a single multi-layer structure. The photosensitive layers in such a multi-layer medium function in principle like the separate media discussed just above in connection with FIG. 1. That is, each layer contains finely-divided photoconductor selectively sensitized to red, green, or blue light. On exposure to radiation such as white light passing through a color negative, the photoconductor is activated in image patterns like those shown in FIG. 1. However, in the multi-layer structure, a different coupler is incorporated into each layer in ballasted form so that a different color is produced within each layer when the exposed medium is contacted with a photographic developer in the presence of a reducing metal ion.

The oxidized developer may react with a ballasted coupler in one of two ways. First, the developer may react with the ballasted coupler to form a diffusible dye, leaving

a non-migrating ballast residue in the layer. Second, a diffusible pre-formed dye, held in a layer by attachment to a ballasting group, may be rendered mobile by reaction of the developer and the ballasting group to release the dye.

Thus, the red-sensitive layer of such a structure may comprise a ballasted coupler forming or releasing a diffusible cyan dye when the coupler is treated with a developer in the presence of metal ion. The green-sensitive

10 layer comprises a ballasted coupler forming or releasing a diffusible magenta dye on reaction with oxidized developer, and the blue-sensitive layer comprises a coupler forming or releasing a diffusible yellow dye on reaction with oxidized developer. The cyan, magenta, and yellow dyes released each diffuse through the layers and are then simultaneously transferred to a receptor sheet by contact processes to form a full-color dye transfer positive print.

The drawing of FIG. 2 shows a multi-layered structure of this type including a support layer suitably of a material such as paper, glass, plastic, or the like. A solution-permeable red-sensitive layer immediately thereover comprises a binder such as gelatin in which is dispersed a finely-divided photoconductor, such as titanium dioxide, which is sensitized to red light with a dye such as taught in Belgian Pat. 714,080. Ballasted couplers forming and/or releasing a cyan dye on development and suitable for inclusion in such a red-sensitive layer are taught, for example, in U.S. Pats. 3,227,551 and 3,243,294.

The red filter layer shown in the structure of FIG. 2 protects the red-sensitive layer from exposure to green and blue light by screening out wavelengths shorter than red.

The green-sensitive layer of the structure of FIG. 2 again comprises a photosensitive photoconductor material such as titanium dioxide, but in combination with a ballasted coupler forming and/or releasing a diffusible magenta dye on reaction with developer in the presence of metal ion at an activated site. Suitable couplers are again those described in U.S. Pats. 3,227,551 and 3,243,294, for example.

40 This layer is protected from wavelengths shorter than green by an overlying yellow filter layer, shown in FIG. 2.

The blue-sensitive layer of FIG. 2 similarly comprises a photoconductive sensitized to blue light with a cyanine or hemicyanine dye like those taught in Belgian Pat. 714,080 and a ballasted coupler forming and/or releasing a diffusible yellow dye at activated sites on reaction with oxidized developer in the presence of metal ion. Such couplers are disclosed, for example, in the U.S. patents mentioned earlier.

50 The multi-layer structure is suitably provided with an abrasion resistant top coat, such as of hardened gelatin, which also controls the diffusion rate of dye from the structure.

After exposure of the multi-layered medium of FIG. 2 to activating radiation, e.g. to white light through a color negative, the exposed medium is suitably developed by first sensitizing it with a reducible metal ion, such as by moistening it with an aqueous solution of silver nitrate. The exposed metal-sensitized medium is then contacted with a developer which, when oxidized, will react with the couplers contained in the different layers of the medium. A variety of alkaline color developing solutions useful for the color development of silver halide media and containing aromatic primary amino color developing agents can be utilized. Particularly useful materials include the p-phenylene diamine color developers.

60 Alternatively the image-forming materials, e.g., solution of metal ions and/or reducing agent therefor may be applied prior to or during exposure.

65 When silver ion is used as the sensitizing metal ion, it is advantageous to separate the development step, i.e. the reaction of silver ion and developer at photo-activated sites to form metallic silver and oxidized developer, from the color coupling step, i.e. the reaction of oxidized developer with coupler to form and/or release a dye. The



Similarly, the exposed red-sensitized film was immediately dipped in a 0.1 N aqueous silver nitrate bath and contacted with a developer solution comprising 0.5 gram of 2-amino-5-diethylamino toluene hydrochloride, 2.0 grams of 1-hydroxy-2-(p-sulfophenyl-N-methyl) naphthamide coupler, 1 gram of hydroxylamine HCl, 15 grams of sodium carbonate, and 0.4 gram of KCNS in 1500 ml. of water.

The coupler,



was prepared as follows.

17.5 g. of N-methylsulfanilic acid sodium salt and 17.3 g. of 1-hydroxy-2-naphthoylchloride were combined in 190 cc. of dry pyridine and refluxed for 3 hours. The hot solution was filtered to remove a small amount of insoluble salt. The solution was cooled and 300 cc. of ether were added. A precipitate formed and the mixture was left standing over the weekend. The precipitate was filtered off and washed with acetone. After drying, 27 g. of white crystals were obtained, which were dissolved in 80 cc. of H<sub>2</sub>O. The solution was made alkaline with Na<sub>2</sub>CO<sub>3</sub> solution and after addition of NaCl a heavy crystalline precipitate formed. After standing for one-half hour in a refrigerator, the precipitate was filtered off and washed first with salt water, followed by H<sub>2</sub>O, and finally with acetone. After drying, 19 g. of product were obtained and dissolved in 400 cc. of boiling methanol. The solution was filtered hot and concentrated to 300 cc. After standing in the refrigerator overnight the product was filtered off, washed with methanol and dried. Yield: 13 g. M.P. 317-318° C.

The resulting cyan image was transferred to the same receptor sheet in register with the magenta image.

Finally, the exposed blue-sensitized film was contacted with silver nitrate and then with a developer solution containing N,N-diethyl-p-phenylenediamine developer and sulfobenzoylacetanilide as the coupler.

The coupler,



is prepared from ethyl benzoylacetate and sodium sulfanilate.

#### EXAMPLE 5

##### Preparation of a multi-layered copy medium

A multi-layered copy medium like that shown in FIG. 2 is prepared by coating a sheet of subbed cellulose triacetate with a first photosensitive layer comprising a ballasted cyan-forming coupler in combination with a finely-divided photoconductor, titanium dioxide, appropriately sensitized to red light.

Specifically, a gelatin layer containing photosensitive titanium dioxide, like the layer described in Example 1 herein, was prepared and deposited on a support layer. The gelatin layer was sensitized to red light by incorporating therewith a red-sensitizing dyestuff of the type taught in Example 2. Also incorporated in the gelatin was a non-diffusing cyan coupler capable of reaction with oxidized color developer to release a diffusible pre-formed cyan dye.

In particular, the non-diffusing cyan coupler had the following structure:



Alternatively, one of the ballasted couplers taught in columns 17-20 of U.S. Pat. 3,227,551 can be incorporated in this layer. These couplers, however, react with oxidized developer to form a diffusible cyan dye rather than to release a pre-formed dye.

A gelatin filter layer containing a water-soluble non-diffusing red azo dye of the formula



was next applied over the red-sensitive layer.

A green-sensitive layer is then applied over the red filter layer. The green-sensitive layer is prepared from a gelatin solution containing finely-divided green-sensitized titanium dioxide and a non-diffusing coupler capable of reacting with oxidized developer to release a pre-formed magenta dye.

Specifically, the coupler used had the following formula:



Alternatively, one of the ballasted couplers taught in column 21 or 22 of U.S. Pat. 3,227,551 can be incorporated into this layer. These couplers react with oxidized developer to form a diffusible magenta dye rather than to release a preformed dye.

A yellow filter layer is next laid atop the green-sensitive layer. The yellow dye of this filter layer may have the following structure, for example:



A blue-sensitive layer containing gelatin and finely-divided titanium dioxide as earlier described herein, is next applied. The photoconductor pigment is sensitized to blue light with a dye as described in Example 2, and the layer additionally contains a non-diffusing coupler releasing a preformed diffusible yellow dye or forming a diffusible yellow dye on reaction with oxidized developer. U.S. Pat. 3,227,551 teaches ballasted couplers releasing a diffusible pre-formed yellow dye in columns 12-15, for example, and couplers forming a diffusible yellow dye in column 23.

Finally, an abrasion-resistant gelatin topcoat is applied over the blue-sensitive layer.

A full color positive print is made by exposing the above-described copying medium to a source of white light through the negative image to be copied.

The exposed medium is then contacted with aqueous silver nitrate and a conventional color developing solution containing an aromatic primary amino developing agent, preferably under acid conditions which promote maximum silver densities but inhibit color coupling. For example, the developing solution can comprise a mixture of silver nitrate and a developer such as 4-amino-N-ethyl-N-β-hydroxy-ethyl aniline sulfate, acidified with acetic acid. In each of the light-sensitive layers of the exposed printing medium which have been struck by light, the activated photoconductor effects reduction of the silver ion to metallic silver and oxidation of the developer.

When the developed medium is next treated in an alkaline bath, the oxidized developer reacts with the ballasted couplers present in the various layers, and forms and/or releases diffusible cyan, magenta, and yellow dyes from these layers.

The diffusible dyes are transferred by contact of the developed multi-layer medium with an appropriate printing paper, for example a receptor sheet of the type earlier described herein.

#### EXAMPLE 6

##### Fog reduction by competing couplers

To reduce fog-producing dye density in unexposed areas of the multi-layer medium described in the previous example, a fast-acting competing coupler such as α-naphthol may be included in the photosensitive layers with the ballasted couplers. For example, α-naphthol may be imbibed into the gelatin layers of the medium by one-minute's immersion in a weakly basic dilute (about 0.1%) solution of naphthol.

In those portions of the medium irradiated during exposure, the amount of competing coupler is small in comparison with the amount of oxidized developer produced in the presence of radiation-activated photoconductor. Accordingly, the ballasted couplers react in normal fashion in these areas to produce diffusible dyes. In non-irradiated areas where, nevertheless, oxidized developer may be produced by an unwanted reaction of developer with silver ion, the competing coupler reacts quickly with any oxidized developer produced to form a non-diffusing product. The amount of oxidized coupler in inactivated areas is small and is consumed by reaction with the fast-reacting competing coupler in preference to reaction with the ballasted coupler. The competing coupler thus ties up the oxidized developer, preventing dye production by its reaction with the ballasted couplers. In this way, a dye image is still produced in light-struck areas, while fog dye

75

density in non-exposed areas is reduced by the formation of non-diffusible substances.

What is claimed is:

1. A photographic imaging medium for making positive full-color dye-transfer prints, said medium comprising a support layer having thereon a plurality of radiation-sensitive layers each comprising a finely-divided reversibly activatable photoconductor, different of said radiation-sensitive layers being sensitized respectively to red, green and blue light and respectively including a different ballasted color coupler generating a cyan, magenta and yellow dye on development, each of said layers also containing a competing, faster-acting coupler forming a non-diffusible product with oxidized developer, and a top coat of hardened gelatin to control the diffusion rate of dye from the medium.
2. A method for forming a full-color, dye-transfer print consisting essentially of:
  - (a) exposing red-, green-, and blue-sensitized photographic imaging media to imaging radiation from a color master, said imaging media each comprising a finely-divided reversibly activatable photoconductor which is reversibly activatable by imaging radiation dispersed in a gelatin binder;
  - (b) developing under acidic conditions each of said imaging media in the presence of silver ions with a silver reducing agent and color coupler to thereby develop a silver image while simultaneously preventing color coupling;
  - (c) contacting said imaging medium with an alkaline solution to cause color coupling thereby generating diffusible cyan, magenta and yellow dye images in radiation-exposed portions of said respective media; and,
  - (d) transferring in register said cyan, magenta and yellow dye images to a receptor to form said full-color print.
3. A method of claim 2 wherein said imaging media contain color couplers in ballasted form, the couplers in said red-, green-, and blue-media respectively generating diffusible cyan, magenta and yellow dyes upon reaction with developer under alkaline conditions.
4. A method of claim 3 wherein a second, competing, faster-acting color coupler which forms a non-diffusible product upon reaction with developer is additionally present in said radiation-sensitive layers during development.
5. A method of claim 4 wherein said receptor comprises a mordanted receptor sheet.
6. A method of claim 5 including the additional step of hardening gelatin layers in said imaging media prior to transferring dye to said receptor sheet.
7. A method of claim 6 including the additional step of rinsing the imaging media in dilute acetic acid after color coupling but prior to transfer of the cyan, magenta and yellow dyes.
8. A method of claim 7 wherein said competing coupler comprises α-naphthol.
9. A method for forming a color dye-transfer print consisting essentially of:
  - (a) exposing a photographic imaging medium to actinic radiation, said imaging medium comprising a finely-divided reversibly activatable photoconductor which is reversibly activatable by actinic radiation;
  - (b) developing under acidic conditions the exposed portions of said medium in the presence of silver ions, a silver reducing agent and a color coupler to thereby develop a silver image while simultaneously preventing color coupling;
  - (c) contacting exposed portions of said medium with an alkaline solution to cause color coupling thereby generating a diffusible dye image in radiation-exposed portions; and,
  - (d) transferring said dye image to a receptor to form a positive color print.

## 11

## References Cited

## UNITED STATES PATENTS

- 3,329,590 7/1967 Renfrew ----- 204-18  
 3,390,989 7/1968 Berman ----- 96-27  
 3,345,163 10/1967 Land et al. ----- 96-3  
 3,320,062 5/1967 Land et al. ----- 96-3  
 2,848,326 8/1958 Whitmore ----- 96-44  
 2,774,668 12/1956 Rogers ----- 96-29  
 2,647,049 7/1953 Land ----- 95-2

10

## FOREIGN PATENTS

- 1,043,250 Great Britain ----- 96-27

## 12

## OTHER REFERENCES

- Collins and Giles, The Journal of the Society of Dyers and Colourists, vol. 68, No. 11, p. 448, 1952.  
 Color Photography, Kirk-Othmer Encyclopedia of Chemical Technology, 2nd ed., vol. 5, p. 819.

CHARLES E. VAN HORN, Primary Examiner  
 M. B. WITTENBERG, Assistant Examiner

## U.S. CL. X.R.

96-1 R, 1.5, 27, 69, 74